

## [54] PERMANENT PRESS TEXTILE FINISH

- [75] Inventors: **William Frank Herbes**, Bridgewater Township, Somerset County, N.J.; **Robert George Weyker**, Memphis, Tenn.
- [73] Assignee: **American Cyanamid Company**, Stamford, Conn.
- [22] Filed: **Apr. 16, 1973**
- [21] Appl. No.: **351,395**

## Related U.S. Application Data

- [63] Continuation-in-part of Ser. No. 124,910, March 16, 1971, abandoned, which is a continuation of Ser. No. 763,344, Sept. 27, 1968, abandoned.
- [52] U.S. Cl. .... **427/390**; 8/186; 427/392
- [51] Int. Cl.<sup>2</sup> ..... **D06M 15/12**
- [58] Field of Search ..... 117/143 A, 145, 139.4, 117/139.5 A; 260/29.4 R, 849; 8/186

## [56] References Cited

## UNITED STATES PATENTS

- |           |        |                     |             |
|-----------|--------|---------------------|-------------|
| 2,731,364 | 1/1956 | Reibnitz et al..... | 117/139.4 X |
| 3,079,279 | 2/1963 | Van Loo.....        | 117/139.4   |
| 3,335,113 | 8/1967 | Dundon .....        | 117/143     |

Primary Examiner—Thomas J. Herbert, Jr.

Assistant Examiner—Bruce H. Hess

Attorney, Agent, or Firm—H. G. Jackson

## [57]

## ABSTRACT

Crease-resistant finishes for cellulosic fibers, said finishes containing 1,3-dimethylol-4,5-dihydroxyethyleneurea and up to 60% urea-formaldehyde condensation products, said finishes being resistant to the degradation effects of chlorine.

7 Claims, No Drawings

## PERMANENT PRESS TEXTILE FINISH

This application is a continuation-in-part of Application Ser. No. 124,910 filed Mar. 16, 1971, now abandoned, which is a continuation of application Ser. No. 763,344 filed Sept. 27, 1968, now abandoned.

This invention relates to crease-resistant aminoplast textile finishes for cellulosic fibers. More particularly, it relates to aqueous aminoplast textile finishes containing 1,3-dimethylol-4,5-dihydroxyethyleneurea and urea-formaldehyde condensation products, to the method of applying the finishes and to the textile materials thus obtained.

1,3-Dimethylol-4,5-dihydroxyethyleneurea (i.e., 1,3-dimethylol-4,5-dihydroxy-2-imidazolidinone) is a known aminoplast agent for finishing textile materials, particularly cellulosic textile materials, in order to obtain wash-and-wear and durable-press properties as disclosed in U.S. Pat. No. 2,731,364, for example. The finish not only gives good wrinkle resistant properties, but also does not cause yellowing or degradation of cellulosic fabrics in the presence of chlorine. The preparation of 1,3-dimethylol-4,5-dihydroxyethyleneurea requires the use of glyoxal, which is a relatively expensive intermediate as compared with the majority of intermediates used in preparing other crease-resistant textile finishes. However, none of the conventionally used, less expensive crease-resistant textile finishes have been found to be equal to 1,3-dimethylol-4,5-dihydroxyethyleneurea in all respects. A need exists, therefore, for a textile finish which will perform as well as 1,3-dimethylol-4,5-dihydroxyethyleneurea and yet be less costly to manufacture.

It is therefore an object of this invention to provide a relatively inexpensive, effective permanent-press textile finish which is resistant to the degradation effects of chlorine.

A further object is to provide such a finish for use on textiles to be subjected to laundering and bleaching.

These and other objects of the invention will become apparent as the description thereof proceeds.

A crease-resistant finish for cellulosic textile materials has now been discovered which is essentially equal to 1,3-dimethylol-4,5-dihydroxyethyleneurea in all respects and at the same time is more economical than the dihydroxyethyleneurea compound. The textile finish of this invention is an aqueous solution of a mixture of 1,3-dimethylol-4,5-dihydroxyethyleneurea and a urea-formaldehyde condensate as defined below.

The urea-formaldehyde condensates are considerably cheaper to manufacture than 1,3-dimethylol-4,5-dihydroxyethyleneurea. However, it is well-known that urea-formaldehyde condensates cause considerable loss in strength of the fabric when the fabric is treated with chlorine, as in a laundering operation, followed by pressing with a hot iron. The strength loss is usually termed "degradation due to chlorine retention."

Therefore, it is very surprising that a considerable portion of the 1,3-dimethylol-4,5-dihydroxyethyleneurea normally used in a textile finish can be replaced by a urea-formaldehyde condensate without materially increasing the strength loss due to chlorine retention.

Various methods have been disclosed for the manufacture of 1,3-dimethylol-4,5-dihydroxyethyleneurea. All the procedures use urea, glyoxal and formaldehyde with variations in the reaction conditions as disclosed

in U.S. Pat. Nos. 2,731,472; 2,764,573 [combination of the two patents], 2,876,062; 3,049,446; and British Pat. No. 1,032,379.

The urea-formaldehyde condensates of use in this invention are the reaction products of urea with formaldehyde, i.e., they are polymethylol derivatives of urea. The condensates should contain at least 1.8 moles, preferably between 2.0 and 3.6 moles, of combined formaldehyde per mole of urea. (4.0 Moles of formaldehyde per mole of urea is the theoretical maximum amount of combined formaldehyde). The use of products containing more than 3.6 moles of formaldehyde per mole of urea is not desirable since it may decrease the stability of the textile finish. The urea-formaldehyde condensates may be partially alkylated if desired, but it is not necessary. The solubility of the lower methylolation products is increased by partial alkylation, preferably methylation, by well-known procedures. Particularly suitable urea-formaldehyde condensates for use in this invention are: (1) a condensate containing 2.8 moles of combined formaldehyde per mole of urea with a slight degree of methylation and (2) a condensate containing about 3.4-3.5 moles of combined formaldehyde, as disclosed in U.S. Pat. No. 3,335,113.

The urea-formaldehyde condensates used in the textile finish of this invention may be employed in amounts up to 60%, preferably up to 50%, of the combined aminoplast components of the textile finish. The lower limit is 5% and preferably 25% on an economical basis, although there is no lower limit as far as effectiveness goes.

The amount of combined aminoplast components of the finish applied to the cellulosic textile materials should be between 2 and 20%, preferably between 3 and 10%, o.w.f. (on weight of fabric). The application is by conventional methods from an aqueous medium as by padding, spraying, dipping, etc.

The treated fabrics are dried and then "cured," or dried and "cured," at an elevated temperature, normally between 250° and 375°F., preferably between 300° and 350°F. Curing at the higher end of the temperature range often provides superior results.

It is recommended that a curing catalyst be used to accelerate the cure of the finish on the fabric. Conventional acid-acting catalysts may be used and they are conveniently applied to the fabric simultaneously with the aminoplast finish from the same padding bath. Such catalysts are well-known, for example, as disclosed in U.S. Pat. No. 3,079,279. The preferred catalyst is zinc nitrate. Conventional amounts are used, i.e., in the range of 5 to 15% based on the combined aminoplast components.

Cellulosic textile materials include cotton, rayon (re-generated cellulose), linen, and other materials containing cellulosic fiber. It also includes blends of cellulosic fibers and other fibers, such as the synthetic fibers, e.g., nylons, polyesters, polyacrylonitriles, etc. The blend should contain at least 20%, preferably at least 30%, of cellulosic fibers.

The following specific examples are given to illustrate the invention and are not intended to be limitative.

## EXAMPLE 1

Five pad baths were prepared containing the relative amounts of 1,3-dimethylol-4,5-dihydroxyethyleneurea

("Resin A") and a slightly methylated urea-formaldehyde condensate having about 2.8 moles of combined formaldehyde per mole of urea ("Resin B") shown in Table I, each bath containing 5.75% (by weight) of total "resin" solids and 10% of zinc nitrate based on the "resin" solids.

The pad baths were applied to 80 × 80 cotton percale by a standard padding procedure obtaining an 80% wet pick-up. The treated fabrics containing 4.6% of total "resin" solids were dried at 225°F. for 2.0 minutes and then heated at 350°F. for 1.5 minutes.

Swatches of untreated and treated fabrics were tested for wrinkle recovery by Tentative Test Method AATCC 66-1959T.

Strength loss of the fabrics due to retained chlorine was measured by Standard Test Method AATCC 92-1967 after 5 washes in a home-style washing machine using water at 140°F. and a synthetic detergent.

The results are shown in Table I.

TABLE I

|    | Resin A<br>% | Resin B<br>% | Total Wrinkle<br>Recovery<br>Degrees, W + F | Strength<br>Loss Due<br>to Chlorine<br>Retention, % |
|----|--------------|--------------|---------------------------------------------|-----------------------------------------------------|
| a. | 100          | 0            | 282                                         | 12                                                  |
| b. | 70           | 30           | 277                                         | 0                                                   |
| c. | 50           | 50           | 280                                         | 6                                                   |
| d. | 30           | 70           | 284                                         | 37                                                  |
| e. | 0            | 100          | 275                                         | 50                                                  |
| f. | Untreated    |              | 182                                         | 0                                                   |

## EXAMPLE 2

Similar results were obtained when the procedure of Example 1 was repeated using a urea-formaldehyde condensate containing about 3.4 moles of combined formaldehyde per mole of urea.

## EXAMPLE 3

The procedure of Example 1 was followed with the exceptions that the pad baths contained 11.5% of total resin solids, the treated fabrics contained 9.2% resin solids, the fabrics were "cured" at 300°F. for 1.5 minutes, and the fabric washes were carried out with detergent and chlorine (Clorox).

The results of the test are shown in Table II.

TABLE II

|    | Resin A<br>% | Resin B<br>% | Total Wrinkle<br>Recovery<br>Degrees, W + F | Strength<br>Loss Due<br>to Chlorine<br>Retention, % |
|----|--------------|--------------|---------------------------------------------|-----------------------------------------------------|
| a. | 100          | 0            | 301                                         | 14                                                  |
| b. | 70           | 30           | 300                                         | 11                                                  |
| c. | 50           | 50           | 299                                         | 15                                                  |
| d. | 30           | 70           | 292                                         | 39                                                  |
| e. | 0            | 100          | 293                                         | 52                                                  |
| f. | Untreated    |              | 182                                         | 0                                                   |

Seven pad baths were prepared containing the relative amounts of 1,3-dimethylol-4,5-dihydroxyethyleneurea ("Resin A") and a slightly methylated urea-formaldehyde condensate having about 2.8 moles of combined formaldehyde per mole of urea ("Resin B") shown in Tables III and IV, each bath containing 5.29% (by weight) of total resin solids and 10% of zinc nitrate based on the resin solids.

The pad baths were applied to 80 × 80 cotton percale by a standard padding procedure obtaining an 87% wet pick-up. The treated fabrics containing 4.6% of total resin solids were dried at 225°F. for 2.0 minutes and then heated: (a) at 350°F. for 1.5 minutes and (b) at 300°F. for 1.5 minutes; see Tables III and IV, respectively. Swatches of untreated and treated fabrics were tested for wrinkle recovery by Tentative Test Method AATCC 66-1959T. Strength loss of the fabrics due to retained chlorine was measured by Standard Test Method AATCC 92-1967 after 5 washes in a homestyle washing machine using water at 140°F. with a synthetic detergent and Clorox.

The two sets of test data shown for each application in Tables III and IV represent physical tests measured on randomized duplicates submitted from each treatment. These data demonstrate that low losses in strength due to chlorine retention are obtained at levels of 0-70% of Resin B when the cure is carried out at 350°F.

TABLE III

|    | (cured 1.5 mins. at 350°F) |              |                                           | Strength<br>Loss Due<br>to Chlorine<br>Retention, % |      |
|----|----------------------------|--------------|-------------------------------------------|-----------------------------------------------------|------|
|    | Resin A<br>%               | Resin B<br>% | Total Wrinkle<br>Recovery<br>Degrees, W/F |                                                     |      |
| 25 | a.                         | 100          | 0                                         | 303                                                 | 0.0% |
|    | b.                         | 95           | 5                                         | 288                                                 | 7.6% |
|    | c.                         | 85           | 15                                        | 295                                                 | 3.5% |
|    | d.                         | 70           | 30                                        | 301                                                 | 0.0% |
|    | e.                         | 50           | 50                                        | 301                                                 | 7.1% |
|    | f.                         | 30           | 70                                        | 296                                                 | 3.3% |
|    | g.                         | 0            | 100                                       | 290                                                 | 3.4% |
|    | h.                         | Untreated    |                                           | 280                                                 | 3.2% |

TABLE IV

|    | (cured 1.5 mins. at 300°F) |              |                                           | Strength<br>Loss Due<br>to Chlorine<br>Retention, % |       |
|----|----------------------------|--------------|-------------------------------------------|-----------------------------------------------------|-------|
|    | Resin A<br>%               | Resin B<br>% | Total Wrinkle<br>Recovery<br>Degrees, W/F |                                                     |       |
| 50 | a.                         | 100          | 0                                         | 287                                                 | 2.9%  |
|    | b.                         | 95           | 5                                         | 287                                                 | 3.0%  |
|    | c.                         | 85           | 15                                        | 290                                                 | 2.8%  |
|    | d.                         | 70           | 30                                        | 285                                                 | 0.0%  |
|    | e.                         | 50           | 50                                        | 279                                                 | 0.0%  |
|    | f.                         | 30           | 70                                        | 285                                                 | 2.8%  |
|    | g.                         | 0            | 100                                       | 280                                                 | 8.3%  |
|    | h.                         | Untreated    |                                           | 277                                                 | 27.7% |

While we have set forth certain specific embodiments and modes of practice of the invention, it will be understood that this is solely for the purpose of illustration and that various changes and modifications may be made without departing from the scope of the disclosure or spirit of the appended claims.

We claim:

1. A method for providing a crease resistance to cellulosic-containing textile materials which comprises

applying from about 2 to 20%, based on the weight of said textile materials of an aminoplast finish comprising an aqueous solution of a mixture of 1,3-dimethylol-4,5-dihydroxyethyleneurea and a urea-formaldehyde condensate, said urea-formaldehyde condensate being from 5 to 50% by weight of the total aminoplast and said 1,3-dimethylol-4,5-dihydroxyethyleneurea being from 50 to 95% of the total aminoplast, said urea-formaldehyde condensate further containing from 1.8 to 3.6 mols of combined formaldehyde, thereafter drying said textile material and curing said finish on said textile at an elevated temperature, in the presence of an acid acting catalyst.

2. A cellulose containing material having an aminoplast crease resistant finish cured thereon, said finish comprising from about 2 to 20%, based on the weight of said material, of a mixture of 1,3-dimethylol-4,5-dihydroxyethyleneurea and a urea-formaldehyde condensate, said condensate having from 1.8 to 3.6 mols of combined urea and being from about 5 to 50% of said finish and said 1,3-dimethylol-4,5-dihydroxyethyleneurea being from 50 to 95% of said finish.

3. A method according to claim 1 wherein the urea-formaldehyde condensate is from 5 to 30% by weight of the total aminoplast and the 1,3-di-methylol-4,5-

dihydroxyethyleneurea is from 95 to 70% by weight of the total aminoplast.

4. A method according to claim 3 which comprises applying about 4.6%, based on the weight of said textile materials, of an aminoplast comprising an aqueous solution of a mixture of 1,3-dimethylol-4,5-dihydroxyethyleneurea and a urea-formaldehyde condensate, said urea-formaldehyde condensate being about 70% by weight of the total aminoplast and said 1,3-dimethylol-4,5-dihydroxyethyleneurea being about 30% by weight of the total aminoplast, said urea-formaldehyde condensate containing about 2.8 mols of combined formaldehyde.

5. A method according to claim 4 comprising drying said textile material at about 225°F. for about 2.0 minutes and curing said dried textile material for about 1-5 minutes at 350°F.

6. A material according to claim 2 wherein the urea-formaldehyde condensate is from 5 to 30% by weight of the total aminoplast and the 1,3-dimethylol-4,5-dihydroxyethyleneurea is from 95 to 70% by weight of the total aminoplast.

7. A cellulose containing textile material finished according to the method of claim 4.

\* \* \* \* \*

30

35

40

45

50

55

60

65